

Patented Nov. 6, 1923.

1,472,882

# UNITED STATES PATENT OFFICE.

HERBERT RAYMOND MOODY, OF NEW YORK, N. Y.

## PROCESS OF MAKING OILS NONSLUDGING.

No Drawing.

Application filed February 6, 1918. Serial No. 215,715.

To all whom it may concern:

Be it known that I, HERBERT R. MOODY, a citizen of the United States, residing at No. 330 Convent Avenue, New York city, in the 5 county of New York, State of New York, have invented certain new and useful Improvements in Processes of Making Oils Nonsludging; and I do hereby declare the following to be a full, clear, and exact description of the invention, such as will enable others skilled in the art to which it 10 pertains to make and use the same.

This invention relates to the treatment of 15 unsaturated organic liquids, and particularly to the treatment of petroleum fractions, having definite electrical mechanical and chemical properties, in order to make them "non-sludging" when subjected (with or without contact with copper or other metal) 20 to an oxidizing heat treatment.

In oils such as are used, for example, in electrical transformers, or such as are used as insulating or cooling liquids, or for 25 lubrication in various forms of electrical or mechanical apparatus, it is important that the oils should not "sludge." The common methods of purifying such petroleum fractions do not free them from sludge-forming constituents, and, upon use under 30 conditions where they are subjected to heat and to oxidation, such oils frequently have sludge of an objectionable nature formed therein.

It is an object of the present invention 35 to remove from such oils their sludge-forming constituents and properties, and to impart to the oils improved properties and qualities which adapt them particularly for use for purposes such as those noted above.

According to the present invention, the 40 oil, such as petroleum fraction of a consistency adapted for the intended purpose, after proper fractionation, filtration, or other clarification treatment, is digested 45 with caustic alkali and with an appropriate metal in a suitable state of subdivision or comminution. It has been found that in practice the best metals are those which are the most electro-negative to the alkali 50 metals and form salts therewith. Among these metals may be mentioned zinc, which forms zincates, aluminum which forms aluminates, iron which forms ferrates, tin which forms stannates, etc. Scrap tinned 55 iron plate is also available for use. The oil, caustic alkali, and metal, are heated to

the appropriate temperature for a sufficient time to enable the desired action to take place, the action being promoted, if desired, by continuous agitation, or by otherwise 60 bringing the oil into intimate contact with the metal and alkali. After the treatment, the salts formed can be separated from the oil in any suitable manner, as by washing, and should in practice be separated where 65 their presence would be detrimental in the treated oil, for example, where their presence would decrease the electrical resistance of oil intended for insulating purposes.

The action can be further promoted by 70 the presence of metals which do not combine with the alkali metals in the manner above indicated but which act catalytically, and thereby facilitate or promote the desired reaction. Among such catalytic metals 75 may be mentioned nickel, copper, metals of the platinum group, etc. These metals may be in a finely divided form, or may be spread upon various inert supports. Metals which are formed by reduction of their oxides, 80 such as reduced nickel, are of particular value, because of their high catalytic efficiency. So also, catalytic metals otherwise prepared and possessing high catalytic efficiency can be used to advantage. It is also 85 preferable to carry out the reaction in iron vessels, rather than glass vessels.

The invention will be further illustrated 90 by the following more detailed description of a specific embodiment thereof.

A suitable petroleum fraction, such as is used for lubricating or electrical purposes, and which has been freed from the gasoline and benzine fractions, and from the lighter illuminating oils, is agitated with the caustic 95 alkali and metal in a suitable receptacle, which may be provided with a steam jacket or other heating means, and with an agitator or stirrer for causing the agitation of the oil. Thus, to 100 liters of oil about 1.7 100 kilos of finely divided aluminum, e. g., aluminum powder, and about 5 kilos of caustic soda, are added, and the mixture is suitably agitated and heated to from 70° to 120° C., preferably at from 90° to 100° 105 C. The caustic soda is used in considerable excess of that which is theoretically necessary. The temperature is maintained approximately constant until the desired reaction has been effected and the sludge-forming constituents have been modified and 110 thus eliminated or converted into non-

sludging constituents. This usually requires several hours, and may require a day or more.

The reaction which takes place in the process above described is a reduction reaction, the caustic alkali and the aluminum combining with the evolution of hydrogen, in a nascent condition, within the body of the oil. The setting free of this hydrogen in a peculiarly reactive form, and within the oil body, enables the reduction or saturation of the unsaturated bodies present to take place in an advantageous manner. This action may, in some cases (as with zinc) be promoted by the presence of a catalytic metal, such as catalytically active nickel.

At the end of the process the metal remaining as such, and the salts formed, can be removed by settling, or by filtering, or by washing, or otherwise. The oil is thus obtained free from the reagents with which it has been treated, and freed also by the treatment from its sludge-forming constituents. These constituents, of an unsaturated nature, are converted during the treatment into the form of saturated bodies, or into bodies of higher saturation, by combining with the hydrogen set free.

Instead of using the caustic alkalis, the alkali carbonates, such as sodium carbonate, may be used, although with less advantage. When using the carbonates, water should also be present, for example, water of crystallization, so that the desired reaction can take place.

Various forms of powdered metal are available for use in the process. Powdered aluminum is particularly valuable. Granular and leaf aluminum do not appear to be so good. When iron is used it may be in the form of a fine powder, or filings, turnings, and the like, or thin sheet iron cut up into small pieces. Tinned scrap iron has the advantage of supplying two metals capable of taking part in the reaction. Metal leaf can also be used with advantage, especially where the metal leaf is in the form of flakes which readily stay in suspension in the oil.

The action of reduction of the unsaturated bodies can be supplemented by the introduction of hydrogen from any suitable external source. This will be of value particularly where a catalytic metal is present to promote the combination of the hydrogen thus added with the unsaturated constituents of the oil, the oil being suitably agitated during the reaction. The present invention accordingly enables the hydrogenation of oils by means of hydrogen gas and a catalytic metal to be further facilitated and promoted by the simultaneous action of the caustic alkali and of the metal which combines therewith with the liberation of nascent hydrogen within the oil mass.

Instead of proceeding in the manner

above described, a similar reaction may be carried out by substituting, for the caustic soda or sodium carbonate, anhydrous aluminum chloride or similarly acting salts, such as ferric or zinc or cuprous chloride, etc. 70 These, at proper temperatures, react with aluminum carbide or other carbides mixed with the oil, when proper sources of combined hydrogen, such as water, are also present, and hydrogen and hydrocarbons 75 are thus evolved.

The conditions favorable for the interaction of these gases and the unsaturated constituents of the oil are readily established, for example, a temperature of 120° to 80 150° C. has been found satisfactory for this reaction.

As a result of this reaction and treatment, the oil can be freed from its propensity to sludge and converted into an oil which 85 yields no sludge.

The novel method of the present invention can be applied to other unsaturated bodies besides those of petroleum fractions, and containing sludge-forming constituents, although the invention is of particular advantage when applied to such petroleum oils. Such petroleum oil fractions, which are otherwise unfitted for certain electrical and mechanical uses because of their sludging propensities, can be thus made practically non-sludging, and can be thus made available for employment in the industries. 95

Among the other unsaturated bodies which can be similarly improved or reduced may be mentioned unsaturated hydrocarbons other than those of petroleum fractions, unsaturated animal and vegetable oils and fats such as the fatty acids and their glycerides, etc. When treating such fatty acids or their glycerides, the temperatures should in general be maintained below those which will cause combination of the alkali with the fatty acid and the formation of soaps, although some formation of soaps may take place simultaneously with the reduction or hardening of the oils. Where soaps are formed during the reaction, they can be removed at the end of the reaction, and used as soap material, or the 100 free fatty acids recovered therefrom. 110

I claim:

1. The process of producing a non-sludging oil from an oil containing sludge-forming constituents, comprising treating the oil with substances which react to evolve hydrogen, the process being carried out at a temperature high enough to cause evolution of hydrogen and a hydrogenation of the sludge-forming constituents of the oil, but 115 not high enough to cause a cracking of the oil being treated. 125

2. The process of producing a non-sludging oil, comprising the step of treating oil with nascent hydrogen, at a comparatively 130

low temperature so that no cracking of the oil takes place, whereby the hydrogen converts the sludge-forming constituents of the oil into non-sludge-forming constituents.

6 3. The process of producing a non-sludging oil, comprising treating an appropriate distillate resulting from the distilling of petroleum, with an alkali and a metal, at a

temperature that is below the cracking temperature of the oil and that causes the alkali and metal to react to form hydrogen, the hydrogen combining with the sludge-forming constituents of the oil to convert them into non-sludge-forming constituents. 10

In testimony wherof I affix my signature.  
HERBERT RAYMOND MOODY.